



US005268118A

**United States Patent [19]**

Bloodworth et al.

[11] Patent Number: 5,268,118

[45] Date of Patent: Dec. 7, 1993

[54] ELECTROVISCOS LIQUIDS BASED ON POLYMER DISPERSIONS WITH AN ELECTROLYTE-CONTAINING DISPERSE PHASE

[75] Inventors: Robert Bloodworth, Cologne; Günther Penners; Günter Oppermann, both of Leverkusen; Roland Flint, Cologne, all of Fed. Rep. of Germany

[73] Assignee: Bayer Aktiengesellschaft, Leverkusen, Fed. Rep. of Germany

[21] Appl. No.: 745,586

[22] Filed: Aug. 15, 1991

[30] Foreign Application Priority Data

Aug. 25, 1990 [DE] Fed. Rep. of Germany ..... 4026881

[51] Int. Cl.<sup>5</sup> ..... C10M 171/00; C10M 169/04  
[52] U.S. Cl. ..... 252/73; 252/74;  
252/572

[58] Field of Search ..... 252/73, 74, 572

[56] References Cited

U.S. PATENT DOCUMENTS

3,970,573 7/1976 Westhaver ..... 252/73  
4,702,855 10/1987 Goosens et al. ..... 252/75  
4,812,251 3/1989 Stangroom ..... 252/75

FOREIGN PATENT DOCUMENTS

0219751 4/1987 European Pat. Off. .  
0284268 9/1988 European Pat. Off. .  
0342041 11/1989 European Pat. Off. .  
0432601 6/1991 European Pat. Off. .  
1-266191 10/1989 Japan .  
2-206692 8/1990 Japan .  
3-035095 2/1991 Japan .

OTHER PUBLICATIONS

Matsepuro, "Structure Formation in an Electric Field and the Composition of Electrorheological Suspensions", Translated from Elektroreol. Issled Pril, Minsk, pp. 27-51, 1981.

Primary Examiner—Christine Skane

Attorney, Agent, or Firm—Sprung Horn Kramer & Woods

[57] ABSTRACT

The present invention relates to electroviscous liquids consisting essentially of  
(I) a polymer or polymer mixture,  
(II) an electrolyte dissolved in (I),  
(III) optionally an additive miscible with the solution of (I) and (II),  
(IV) optionally a viscosity-increasing additive reacting with (I);  
(V) a dispersant and  
(VI) a non-aqueous dispersion medium.

7 Claims, 3 Drawing Sheets





FIG.1



Fig. 2



Fig. 3

## ELECTROVISCOS LIQUIDS BASED ON POLYMER DISPERSIONS WITH AN ELECTROLYTE-CONTAINING DISPERSE PHASE

### BACKGROUND OF THE INVENTION

This invention relates to an electroviscous liquid which undergoes an increase in viscosity on application of a voltage.

Electroviscous liquids (EVLs) are dispersions of fine-particle solids in hydrophobic and electrically non-conductive oils of which the viscosity may be increased very quickly and reversibly from the liquid to the plastic or solid state under the effect of a sufficiently strong electrical field. Their viscosity responds both to electrical d.c. fields and to a.c. fields, the current flowing through the EVL having to be extremely low. Accordingly, EVLs may be used for any applications in which it is desired to control the transmission of powerful forces by low electric power levels, for example in clutches, hydraulic valves, shock absorbers, vibrators or systems for positioning and holding workpieces in position.

In addition to the requirements which an EVL generally has to satisfy, such as a good electroviscous effect, high temperature stability and chemical stability, the abrasiveness and sedimentation stability behavior of the disperse phase play an important part in practical application. Ideally, the disperse phase should not sediment, but at all events should be readily redispersible and should not cause any abrasion under extreme mechanical stressing.

In qualitative terms, the increase in viscosity which an EVL undergoes on application of an electrical field may be explained as follows: the colloidally stable disperse particles polarize in the electrical field and agglomerate through dipole interaction in the direction of the field, resulting in the increase in viscosity. The agglomeration is reversible: if the electrical field is switched off, the particles redisperse and viscosity is reduced to the original value. The polarizability of the disperse phase is thus an important requirement for the development of an electroviscous effect. For this reason, ionically or electronically conductive materials are often used as the disperse phase.

In some of the EVLs corresponding to the prior art, the disperse phase consists of organic solids, such as for example saccharides (DE 2 530 694), starch (EP 2 842 268 A2, U.S. Pat. No. 3,970,573), polymers (EP 150 994 A1, DE 3 310 959 A1, GB 1,570,234, U.S. Pat. No. 4,129,513, ion exchanger resins (JP 92 278/975, JP 31 221/1985, U.S. Pat. No. 3,047,507) or silicone resins (DE 3,912 888 A1). However, inorganic materials have also been used, including for example Li hydrazine sulfate (U.S. Pat. No. 4,772,470 A), zeolites (EP 265 252 A2), silica gel (DE 3 517 281 A1, DE 3 427 499 A1) and aluminium silicates (DE 3 536 934 A1).

In the case of the substances mentioned, the electroviscous effect is attributable to the charging of the solids with water. Small water contents increase ionic conductivity and hence the polarizability of the disperse particles which is essential to the development of the effect. However, water-containing systems show poor chemical stability. In addition, the temperature range in which these liquids can be used is limited.

In the case of other electroviscous liquids, efforts have been made to overcome the disadvantages mentioned by replacing the water-containing disperse phase

with a substantially water-free, electronically conductive phase which consists of partly coated, finely disperse metals, such as for example aluminium (JP 016 093, JP 0117 2496), or dielectrics, such as for example  $TiO_2$  (SU 715 596),  $CaTiO_3$  or  $BaTiO_3$  (JP 53/17585), hydrolyzates of metal alkoxides (EP 341 737) or hollow glass bodies (J 0117 2496). However, due to the hardness of the dispersed particles, the described EVLs are abrasive and, hence, are of only limited use for practical applications involving high shear stressing. Carbon-black-filled bead polymers (JP 016 093) or conductive polymers, such as for example polypyrrole or polyacetylene (JP 0126 0710), have also been discussed as substitutes for the water-containing phase.

With the water-containing systems, the optimal properties of the disperse phase can be effectively established by variation of the water content or by modification of the solid matrix. Thus, DE 2 802 494 C2 describes an improvement in the electroviscous effect by introduction of free or neutralized acid groups into a water-containing polymeric phase. In the production of EVLs based on electronically conductive disperse phases, the dispersion particles often had to be aftertreated because of the high electrical conductivity of the starting materials. Thus, JP 016 093 describes the passivation of carbon-black-filled bead polymers by subsequent coating of the polymer particles with polyvinylidene fluoride. However, production costs are greatly increased by aftertreatments of the type in question.

The above-mentioned EVLs corresponding to the prior art are generally produced by dispersion of a solid in a dispersion medium, such as for example halogen-free or halogenated hydrocarbons, aromatic hydrocarbons or silicone oil. The viscosity of the suspension formed depends upon the shape and size or size distribution of the dispersed particles and upon the solids concentration and dispersion effect of any dispersion aids used. High volume-related solids contents for low viscosities are difficult to achieve where non-spherical particles are used.

The problem addressed by the present invention was to provide a water-free, non-abrasive, non-sedimenting EVL having good electroviscous properties which would be distinguished by a low basic viscosity despite a high content by volume of disperse phase.

### DESCRIPTION OF THE INVENTION

It has been found that electroviscous liquids of the type in question can be produced on the basis of anhydrous polymers containing dissolved electrolyte. The electroviscous properties of these liquids can be adjusted as required over wide ranges through the type and concentration of the electrolyte. In addition, the electroviscous dispersions according to the invention are water-free and show high dielectric strength. Another advantage to be emphasized is that the described EVLs are sedimentation-stable and non-abrasive and show low basic viscosities, despite high contents by volume of disperse phase. The dispersion polymerization of electrolyte-containing monomers is a particularly suitable process for the production of the EVLs according to the invention. Polymerization should preferably be carried out in the dispersion medium, which also represents the continuous phase of the EVLs, because this eliminates the need for subsequent redispersion.

The EVLs according to the invention essentially contain the following substances in the disperse phase: (I) a polymer or polymer mixture, (II) a dissolved electrolyte and, optionally, (III) an additive miscible with the solution of (I) and (II).

The mixture of substances or its starting products are referred to hereinafter as the starting material. The starting material, which is dispersed in the non-conductive liquid during production of the EVLs, should preferably be present in liquid form. The starting material may optionally be chemically modified by the addition of suitable reagents (IV) before, during or after the dispersion step. This modification influences the consistency of the disperse phase in the final EVL by partial or complete reaction of the functional groups in the starting material.

To avoid coalescence where liquid phases are used, a suitable dispersant (V) is used in the dispersion step. The size of the dispersed particles in the EVLs according to the invention is between 0.1 and 200  $\mu\text{m}$ . The viscosity of the EVLs at room temperature is between 3 and 5,000 cp, depending on the composition of the liquid and the basic viscosity of the dispersion medium.

The EVLs according to the invention essentially contain the following substances in the disperse phase: (I) a polymer, (II) a dissolved electrolyte and, optionally, (III) an additive miscible with the solution of (I) and (II).

#### DETAILED DESCRIPTION

Suitable polymers (I) are, in principle, any substances which show electrolyte solubility, such as for example linear or crosslinked polyethers or copolymers thereof, polyethylene adipate, polyethylene succinate and polyphosphazene. However, polyethers or polymers which can be prepared by crosslinking of difunctional or trifunctional polyether oligomers are particularly preferred. Examples of linear polyether oligomers are polyethylene glycols, polypropylene glycols, statistical ethylene/propylene glycol copolymers or even ethylene glycol/propylene glycol block copolymers, for example of the type marketed by GAF under the name "Pluronic". Branched polyether oligomers are, for example, tris(polypropylene oxide) $\omega$ -ol)glycidyl ethers or other substances obtained by ethoxylation of propoxylation of hydroxy compounds of relatively high functionality, such as for example pentaerythritol or 1,1,1-trimethylol propane. The molecular weight of the glycols is between 62 and 1,000,000 and preferably between 100 and 10,000. The oligomers may optionally contain terminal groups. Amines, allyl or vinyl groups or even carboxyl groups are examples of functional terminal groups. Polyethylene or polypropylene monoamines or diamines are marketed by TEXACO under the name "Jeffamin". Examples of products containing vinyl groups are the esters of glycols with corresponding acids, for example acrylic acid. Other preferred polymers are, for example, the polyesters marketed by, among others, BAYER AG under the trade name "Desmophen".

Electrolytes (II) in the context of the invention are substances which are soluble in molecular or ionic form in the polymer (I). Examples of such electrolytes are, for example, free acids or salts thereof with alkali or alkaline earth metals or organic cations. Accordingly, electrolytes include salts such as KCl, LiNO<sub>3</sub>, CH<sub>3</sub>COONa, LiClO<sub>4</sub>, Mg(ClO<sub>4</sub>)<sub>2</sub>, KSCN, LiBr, LiI,

LiBF<sub>4</sub>, LiPF<sub>6</sub>, NaB(C<sub>6</sub>H<sub>5</sub>)<sub>4</sub>, LiCF<sub>3</sub>SO<sub>3</sub>, N(C<sub>2</sub>H<sub>4</sub>)<sub>4</sub>Cl, etc.

Additives (III) according to the invention are compounds which, when mixed with (I) and (II), form a homogeneous, solid or liquid solution. For example, where a polyether is used as the polymer, masked low molecular weight polyethers, such as for example bis-methylated trimethylol propane, or the esters of phthalic acid are suitable additives.

Where liquid starting materials are used, an additive (IV) (for example a crosslinking agent) is optionally added to the system before or after emulsification of the starting material and, by reaction with the functional terminal groups in the compounds (I), leads to an increase in molecular weight in the emulsion droplets or even to a reduction in the number of functional terminal groups. Depending on the type and quantity of the mixture components and additives used, viscous or solid particles are formed, retaining their spherical geometry during and after the reaction.

Where the starting material contains a glycol as component (I), difunctional or multifunctional isocyanates are preferably used as the crosslinking agent (IV). Isocyanates of different structures are marketed by BAYER AG under the name "Desmodur". Where trifunctional or higher glycols are used, it is particularly suitable to use tolylene diisocyanate as the crosslinking agent. However, the acetate, amine, benzamide, oxime and alkoxy crosslinking agents typically used in silicone chemistry may also be used for crosslinking. Radical crosslinking systems are suitable for the reaction of polymer starting materials modified by allyl or vinyl (acryl or methacryl) groups.

The EVLs according to the invention contain from 10 to 95% by weight and preferably from 40 to 70% by weight of the disperse phase (the product of the starting material and (IV)).

Suitable dispersants (V) for the disperse phase are surfactants soluble in the dispersion medium which are derived, for example, from amines, imidazolines, oxazolines, alcohols, glycol or sorbitol. Polymers soluble in the dispersion medium may also be used. Suitable polymers are, for example, polymers containing 0.1 to 10% by weight N and/or OH and 25 to 83% by weight C<sub>2</sub> to C<sub>24</sub> alkyl groups and having a molecular weight in the range from 5,000 to 1,000,000. The N- and OH-functional compounds in these polymers may be, for example, amine, amide, imide, nitrile, 5- to 6-membered N-containing heterocyclic rings or an alcohol and the C<sub>4</sub>-C<sub>24</sub> alkyl groups esters of acrylic or methacrylic acid. Examples of the N- and OH-functional compounds mentioned are N,N-dimethylaminoethyl methacrylate, tert. butyl acrylamide, maleic imide, acrylonitrile, N-vinyl pyrrolidone, vinyl pyridine and 2-hydroxyethyl methacrylate. The polymeric dispersants mentioned above generally have the advantage over the low molecular surfactants that the dispersions prepared with them are more stable in regard to their sedimentation behavior.

However, polysiloxane/polyether copolymers of the type marketed, for example, by GOLDSCHMIDT AG, Essen, FRG, under the name "Tegopren" are preferably used for dispersion in silicone oil. One example of a particularly preferred dispersant for the production of an EVL are polysiloxane polyethers with a ratio by weight of ethylene oxide to propylene oxide of 49:51 which are marketed by GOLDSCHMIDT under the name "Tegopren 5830".

In addition to the polyether polysiloxanes, the reaction products of hydroxyfunctional polysiloxanes with various silanes may be used as dispersants for the production of the EVLs according to the invention. Particularly preferred dispersants from this class of substances are the reaction products of a hydroxyfunctional polysiloxane with aminosilanes.

In addition to liquid hydrocarbons, such as for example paraffins, olefins and aromatic hydrocarbons, silicone oils, such as polydimethyl siloxanes and liquid methylphenyl siloxanes, are preferably used as dispersion medium (VI) for the disperse phase. The silicone oils may be used either individually or in combinations of two or more types. The solidification point of the dispersion media is preferably lower than  $-30^{\circ}\text{C}$ . while their boiling point is above  $150^{\circ}\text{C}$ . The viscosity of the oils at room 20 temperature is between 3 and 300  $\text{mm}^2/\text{s}$ . The low-viscosity oils having a viscosity of 3 to 20  $\text{mm}^2/\text{s}$  are generally preferred because they provide for a lower basic viscosity of the EVLs.

To avoid sedimentation, the oil should also have a density substantially corresponding to the density of the disperse phase. For example, by using fluorine-containing siloxanes either in pure form or in admixture with other silicone oils, it is possible to produce EVLs according to the invention which show no signs of sedimentation for weeks despite a low basic viscosity.

Fluorine-containing siloxanes having the following general structure are particularly suitable for the production of non-sedimenting EVLs:



In a typical method for the production of EVLs according to the invention, the starting material is mixed with the reactive additive or with the crosslinking agent (IV). After homogenization of the components, the mixture is dispersed in a liquid phase containing the dispersant. Shearing homogenizers, high-pressure homogenizers or ultrasound may be used here to achieve a corresponding degree of dispersion. However, dispersion should be carried out in such a way that the particle size does not exceed 200  $\mu\text{m}$ . After dispersion, the product may optionally be left to react out over a prolonged period at a suitable temperature which is typically in the range from 15 to  $150^{\circ}\text{C}$ , depending on the reactivity of the crosslinking agent.

In an alternative method, the crosslinking agent is only incorporated in the dispersion on completion of the dispersion step.

After the reaction, the disperse phase may optionally be separated from the original dispersant and transferred to a new dispersion medium, irrespective of the production method.

In another method of production, the starting material with or without surfactant and the additive (IV) is sprayed to form a fine powder and the powder formed is subsequently dispersed in the liquid phase.

The EVLs thus produced were investigated in a modified rotational viscosimeter of the type described

by W. M. Winslow in J. Appl. Phys. 20 (1949), pages 1137-1140.

The electrode area of the inner rotating cylinder 0.50 mm in diameter measures approx.  $78\text{ cm}^2$  and the gap width between the electrodes is 0.50 mm. For the dynamic measurements, the maximum shear rate may be adjusted to  $2,640\text{ s}^{-1}$ . The maximum measuring range of the shear stress of the viscosimeter is 750 Pa. Both static and dynamic measurements are possible with this modified viscosimeter. The EVLs may be excited both with d.c. and with a.c. voltage.

Where d.c. voltage is used, it may happen with certain liquids that, in addition to the spontaneous increase in viscosity or in the yield point when the field is switched on, the solid particles are also electrophoretically deposited onto the electrode surfaces, particularly at low shear rates or in the case of static measurements. Accordingly, testing of the EVLs is preferably carried out with a.c. voltage and under dynamic shear stress. Readily reproducible flow curves are obtained in this way.

To determine electro-reactivity, a constant shear rate  $0 < D < 2,640\text{ s}^{-1}$  is adjusted and the shear stress  $\tau$  is measured as a function of the electrical field strength  $E$ . With the test apparatus, it is possible to generate alternating fields up to a maximum effective field strength of 2,370 kV/m for a maximum effective current of 4 mA and a frequency of 50 to 550 Hz. However, the measurement is preferably carried out at 50 Hz because the total current is then at its lowest so that the electrical power required is also at its lowest. The flow curves obtained are as shown in FIG. 1. It can be seen that the shear stress  $\tau$  shows a parabolic increase at low field strengths and a linear increase at higher field strengths. The gradient  $S$  of the linear part of the curve is apparent from FIG. 1 and is expressed in  $\text{Pa}\cdot\text{mm}/\text{kV}$ . The threshold value  $E_o$  of the electrical field strength is determined from the point of intersection between the straight line  $S$  and the straight line  $\tau = \tau_o$  (shear stress without an electrical field) and is expressed in kV/m. The increase in the shear stress  $\tau(E) - \tau_o$  in the electrical field  $E > E_o$  may be calculated in accordance with the following equation:

$$\tau(E) - \tau_o = S(E - E_o).$$

The following relation thus applies to the relative increase in viscosity,  $V_r(E)$ , which is obtained by application of an electrical field having a strength  $E$ :

$$V_r(E) = \tau_o(E)/\tau_o = (\tau_o + S(E - E_o))/\tau_o.$$

The relative increase in viscosity determines the switching behavior of an EVL in practice and is therefore an important characteristic along with the absolute effect  $S$ .

#### EXAMPLES

In the following Examples, Comparison Examples 1 to 5 correspond to the prior art. The EVLs described in Comparison Examples 1 to 3 contain as their disperse phase water-containing polymers with free or neutralized acid groups attached thereto by covalent bonds. Comparison Examples 1 to 3 are based on Examples 1, 2 and 7 of DE 2 820 494 C2. The liquids described in these Examples, which are representative of the patent,

have good electroviscous effects, but show high plastic viscosity so that the relative effect is distinctly weaker.

The EVLs described in Comparison Examples 4 and 5 contain as their disperse phase water-free aluminium particles having different coatings. They are taken from Examples 1 and 4 of JP 64-6093. The described EVLs have poor sedimentation properties due to the density and size of the disperse particles ( $>20 \mu\text{m}$ ).

Examples 1 and 10 relate to electroviscous liquids according to the invention. In all the described samples, the average particle diameter is approximately  $2 \mu\text{m}$ . The maximum particle diameter is  $6 \mu\text{m}$ . The samples were measured at a temperature of  $60^\circ\text{C}$ .

The electroviscous properties of the EVLs according to the invention and their viscosity are shown in Table 1. The low basic viscosity of the liquids and the resulting high relative electroviscous effect are particularly emphasized.

The correlation between the electroviscous effect  $S$  and the molar Li component, based on the ethylene oxide content, is shown in the form of a graph in FIG. 2 for LiNO<sub>3</sub>-containing EVLs produced on the basis of crosslinked glycols (Examples 1 to 6).

FIG. 3 shows the trend of the electroviscous effect  $S$  and of the viscosity of an EVL produced in accordance with Example 9 at a shear rate of  $1,000 \text{ s}^{-1}$  as a function of the concentration by weight of the disperse phase. It can be seen that the liquid according to the invention is characterized by low viscosity despite high solids concentrations.

## EXAMPLES

|                    |                                                                                                                                                                        |
|--------------------|------------------------------------------------------------------------------------------------------------------------------------------------------------------------|
| Dispersion medium  | Polydimethyl siloxane (silicone oil)                                                                                                                                   |
|                    | Viscosity at $25^\circ\text{C}$ . $5 \text{ mm}^2/\text{s}$                                                                                                            |
|                    | Density at $25^\circ\text{C}$ . $0.9 \text{ g/cm}^3$                                                                                                                   |
|                    | Dielectric constant $\epsilon_4$ acc. to 2.8                                                                                                                           |
|                    | DIN 53483 at $0^\circ\text{C}/50 \text{ Hz}$                                                                                                                           |
| Dispersed phase    | Trifunctional polyethylene glycol, molecular weight 675, prepared by ethoxylation of trimethylol propane                                                               |
| Dispersant         | Reaction product of 100 parts by weight of an OH-terminated polydimethyl siloxane having a molecular weight of 18,200 and 1 part by weight aminopropyl triethoxysilane |
| Crosslinking agent | Toluylene diisocyanate (TDI)                                                                                                                                           |

### COMPARISON EXAMPLE 1

Example 1 of DE 2 820 494 C2: 30% by volume dispersion of a divinylbenzene-crosslinked polyacrylic acid in a polychlorinated diphenyl fraction. The electroviscous effect at  $30^\circ\text{C}$ . was between 975 and 1,070 Pa·mm/kV, depending on the water content (1.3–5% by weight). The plastic viscosity was 220 mPa.s.  $V_r(3,000)=10.7-12.6$ .

### COMPARISON EXAMPLE 2

Example 2 of DE 2 830 494 C2: 30% by volume dispersion of a divinylbenzene-crosslinked methacrylic acid in a polychlorinated diphenyl fraction. For a water content of <6.2% by weight, the electroviscous effect at  $30^\circ\text{C}$ . measured 690 Pa·mm/kV. The plastic viscosity measured 260 mPa.s.  $V_r(3,000)=8.1$ .

### COMPARISON EXAMPLE 3

Example 7 of DE 2 820 494 C2: 30% by volume dispersion of lithium/chromium polymethacrylate in a polychlorinated diphenyl fraction. In ambient humidity,

the electroviscous effect at  $30^\circ\text{C}$ . measured 1,960 Pa·mm/kV. The plastic viscosity measured 236 mPa.s.  $V_r(3,000)=17.9$ .

### COMPARISON EXAMPLE 4

Example 1 of JP-OS 64-6093: 20% by volume dispersion of an aluminium-oxide-coated aluminium powder in TRIMEX T-08. For a.c. voltage of 60 Hz, the electroviscous effect measured 327 Pa·mm/kV.

### COMPARISON EXAMPLE 5

Example 4 of JP-OS 64-6093: 20% by volume dispersion of an aluminium-oxide-coated aluminium powder in TRIMEX T-08. For an a.c. voltage of 60 Hz, the electroviscous effect measured 371 Pa·mm/kV.

### COMPARISON EXAMPLE 6

In a glass beaker having a nominal volume of 100 ml, 0.6 g of the dispersant are dissolved in 20 g of the dispersion medium. In a second glass beaker, 17.5 g of the glycol are mixed with 6.79 g of the crosslinking agent. For a quantitative reaction, this quantity of crosslinking agent results in stoichiometric reaction of the hydroxyl groups in the glycol and thus corresponds to an OH conversion of 100 mol-%. The reactive mixture of glycol and crosslinking agent is emulsified in the dispersant solution immediately after homogenization with a rotor/stator shearing homogenizer (Ultra-Turrax T25, manufactured by IKA Labortechnik). At a rotational speed of the rotor of 10,000 r.p.m., the emulsification time is 2 minutes. The samples were then fully reacted for 15 hours at  $90^\circ\text{C}$ .

### EXAMPLE 1

An EVL was prepared in the same way as described in Comparison Example 6, except that 0.0273 g solid anhydrous LiNO<sub>3</sub> was dissolved in the glycol before further processing. This corresponds to a molar ratio of Li to EO of 1:1,000, based on the number of ethylene oxide units in the glycol.

### EXAMPLE 2

Preparation as in Example 1, but with 0.109 g LiNO<sub>3</sub> (Li:EO ratio 4:1,000).

### EXAMPLE 3

Preparation as in Example 1, but with 0.218 g LiNO<sub>3</sub> (Li:EO ratio 8:1,000).

### EXAMPLE 4

Preparation as in Example 1, but with 0.328 g LiNO<sub>3</sub> (Li:EO ratio 12:1,000).

### EXAMPLE 5

Preparation as in Example 1, but with 0.564 g LiNO<sub>3</sub> (Li:EO ratio 20:1,000).

### EXAMPLE 6

Preparation as in Example 1, except that 1.253 g nonanoic acid was used as electrolyte (H:EO ratio 2:1,000).

### EXAMPLE 7

Preparation as in Example 1, except that 1.313 g tetraethyl ammonium chloride was used as electrolyte (N(CH<sub>3</sub>CH<sub>2</sub>)<sub>4</sub>:EO ratio 2:1,000).

## EXAMPLE 8

Preparation as in Comparison Example 7, but with 0.0273 g LiNO<sub>3</sub> (Li:EO ratio 2:1,000).

## EXAMPLE 9

3.9 g LiNO<sub>3</sub> were dissolved in 305.46 g glycol. The resulting solution was mixed with 116.4 g crosslinking agent and dispersed in a solution of 6 g dispersant in 200 g silicone oil and further processed as in Comparison Example 6. The solids content of this EVL was adjusted to between 39 and 64% by addition of silicone oil. The trend of the electroviscous effect S and the viscosity of the EVL at a shear rate of 1,000 s<sup>-1</sup> is shown in FIG. 3. 10 15

TABLE 1

| EVL acc. to | Properties             |                 |                   |                               |
|-------------|------------------------|-----------------|-------------------|-------------------------------|
|             | E <sub>o</sub><br>kV/m | S<br>Pa · mm/kV | V(O) mPa.S<br>(1) | V <sub>r</sub> (3,000)<br>(2) |
| Comp. Ex. 6 | 1384                   | 295             | 59                | 9.1                           |
| Example 1   | 738                    | 587             | 63                | 23.5                          |
| Example 2   | 536                    | 707             | 59                | 30.5                          |
| Example 3   | 536                    | 845             | 51                | 41.8                          |
| Example 4   | 560                    | 920             | 40                | 57.1                          |
| Example 5   | 400                    | 990             | 60                | 43.9                          |
| Example 6   | 1228                   | 405             | 51                | 15.0                          |
| Example 7   | 244                    | 841             | 64                | 37.2                          |
| Example 8   | 264                    | 190             | 36                | 15.4                          |

It is understood that the specification and examples are illustrative but not limitative of the present invention and that other embodiments within the spirit and

scope of the invention will suggest themselves to those skilled in the art.

What is claimed is:

1. An electroviscous liquid free of water comprising
  - a) 40 to 70% by weight of a particulate material selected from the group consisting of linear polyethers, branched polyethers, crosslinked polyethers thereof, polyethylene adipate, polyethylene succinate and polyphosphazene, wherein an electrolytic free acid or alkali, alkaline earth metal or organic cation salt thereof, said acid or salt being soluble in the particulate material in molecular or 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995

UNITED STATES PATENT AND TRADEMARK OFFICE  
**CERTIFICATE OF CORRECTION**

PATENT NO. : 5,268,118

DATED : December 7, 1993

INVENTOR(S) : Bloodworth, et al.

It is certified that error appears in the above-indentified patent and that said Letters Patent is hereby corrected as shown below:

Col. 10, lines 7- After " polyethers " insert -- and  
8 oligomers --

Col. 10, line 20 Delete ". " and substitute -- thereof  
or the reaction product of said  
polyether or oligomer with a cross-  
linking agent. --

Signed and Sealed this  
Eighth Day of July, 1997

Attest:



BRUCE LEHMAN

Attesting Officer

Commissioner of Patents and Trademarks